

Nov. 17, 1942.

S. MYERSON

2,302,375

ARTIFICIAL TOOTH AND METHOD OF MAKING THE SAME

Filed March 15, 1940

2 Sheets-Sheet 1



Fig. 1



Fig. 2



Fig. 3



Fig. 4



Fig. 6



Fig. 7

Inventor  
Simon Myerson  
by Robert Ashman & Woodbury  
Atty's.

Nov. 17, 1942.

S. MYERSON

2,302,375

## ARTIFICIAL TOOTH AND METHOD OF MAKING THE SAME

Filed March 15, 1940

2 Sheets-Sheet 2



Fig. 5



Fig. 8



Fig. 10



Fig. 9



13 14 Fig. 11 14 26



Fig. 12 18  
6 Fig. 13



17) 16 Fig. 14 16

Inventor  
Simon Myerson  
by Robert C. Woodbury  
Atty's.

## UNITED STATES PATENT OFFICE

2,302,375

ARTIFICIAL TOOTH AND METHOD OF  
MAKING THE SAME

Simon Myerson, Brookline, Mass.

Application March 15, 1940, Serial No. 324,127

6 Claims. (Cl. 32—10)

This invention pertains to artificial teeth and relates more particularly to improvements designed to impart an appearance more closely simulating that of natural teeth than has heretofore been done, the present application being a continuation-in-part of my copending applications for Letters Patent Serial No. 78,674, filed May 8, 1936; Serial No. 104,039, filed October 5, 1936, now issued as Patent No. 2,202,712; Serial No. 180,725, filed December 20, 1937, now issued as Patent No. 2,202,713 dated May 28, 1940; and Serial No. 191,218, filed February 18, 1938, respectively.

Attempts have previously been made by teeth manufacturers and dentists to make artificial teeth resemble natural teeth in appearance, but despite the most artistic carving and the application of stains and glaze by the dentist, the artificial tooth is readily distinguishable from the normal tooth, at least by experienced persons.

Apparently most previous experiments designed to improve the visual appearance of artificial teeth have been without due regard to the fact that when in use the tooth is viewed against the dark background afforded by the oral cavity, and that the effect of light striking the tooth and being partially reflected therefrom is greatly modified by the presence of this dark background. Failing to recognize this fact, much of the prior experiment and practice has been concerned with the use of colored materials and the application of stains or the like in the effort to obtain the peculiar shadowy effect observed in natural teeth under varying light conditions, but whereas colored material or stain may be effective for the intended purpose under some light conditions they frequently fail utterly to give the desired results under different light conditions, it being well recognized that artificial teeth are particularly noticeable as such at night when observed under artificial light.

While it is a matter of common knowledge that in a very large percentage of natural teeth, the substantially transparent or at least translucent enamel layer not only covers the labial surface of the tooth, but forms in effect a cap at the incisal edge, and that in many instances at least this cap is of substantial depth so that it forms portions of both the labial and the lingual surface of the tooth and extends a substantial distance downwardly beyond the relatively opaque body portion of the tooth, no one, so far as I am aware, has heretofore recognized the fact that this is an important factor in respect to the optical appearance of the natural tooth. More-

over, in the natural tooth, the opaque body portion usually tapers in thickness as it approaches the incisal edge so that its effective opposition to the passage of light gradually diminishes to the point where it merges with the material of the transparent cap. Thus the darkness of the oral cavity is effective not only at the extreme incisal edge but also for a substantial distance (but with diminishing intensity) away from said edge, and this I believe is responsible in large measure for the characteristic appearance of natural teeth as contrasted with that of artificial teeth made in accordance with prior practice.

15. Natural teeth are not of uniform appearance nor are the incisal edge portions of natural teeth (consisting almost wholly of enamel) exactly uniform in color, thickness or texture. As a matter of fact, the labial surface, and in particular the incisal portion of a natural tooth, usually has narrow, more or less parallel faint lines or stains extending substantially perpendicular to the incisal edge, or, in other words, extending lengthwise of the tooth. These narrow lines usually 20 result from the presence of fine cracks in the enamel.

In accordance with the present invention, I construct the artificial teeth as nearly as possible to simulate the construction of the natural teeth 30 as respects the arrangement of the transparent enamel and the relatively opaque body portion, as above described. Thus I cause the body portion to taper downward but to terminate short of the incisal edge, and cause the enamel layer 35 which covers the labial surface of the tooth to form in effect a cap in which the tapered end of the body portion is embedded and which forms the incisal edge and also the lateral edges of the tooth. Thus the transparent material is so 40 blended with the more opaque body material that the finished tooth has a fringe, including the incisal edge, which is preferably of substantially complete transparency, the tooth gradually becoming less transparent toward its mid-portion—the body and gingival portions being as opaque 45 as may be desired.

I also construct the tooth or a tooth facing so 50 that it may be manufactured in finished form and by mass production methods and so that when viewed against the dark background of the oral cavity, it exhibits narrow streaks or shadow lines closely simulating those of natural teeth, the streak-forming material being a permanent part of the tooth structure incorporated during 55 manufacture.

I may also reproduce the effect often found in natural teeth, of an opaque light-colored area distinct from the surrounding portions of the tooth, by embedding in the substance of the tooth a preformed insert of the desired contour so disposed in the mould that it lies close to the labial face of the tooth where it is visible through the enamel. This insert may be of any desired contour and, being of a lighter color than the body portion of the tooth, appears as a whitish irregular area when viewed from the front. By making this insert as a preformed, solid piece, danger of change in shape during the fusing of the tooth may be avoided.

It is common to fill cavities in natural teeth with porcelain fillings, and it has been observed that such fillings in natural teeth commonly bleach during use so as to appear a little lighter than the surrounding material of the natural tooth. Moreover, such porcelain fillings do not always fit snugly, so that it is quite common to observe a stained effect at the junction of the filling with the body of the tooth. Furthermore, such fillings often appear to project slightly from the surface of the tooth itself, both at the labial face and at the incisal edge. In accordance with one aspect of the present invention it is proposed to make an artificial tooth in which the natural appearance is enhanced by giving the tooth an appearance closely simulating that of a natural tooth having a porcelain filling.

In order to obtain an even finer graduation and blending of light effects, it is contemplated that a layer of material, of a transparency intermediate those of the body portion and incisal cap, may be interposed between the labial surface of the tapering part of the body portion and the transparent enamel layer.

The result of the improved construction is that when the tooth is in use and viewed against the dark oral cavity, the incisal portion of the tooth takes on a bluish shadowy appearance, closely simulating the natural tooth, such appearance varying with different light conditions and changes in perspective as it does in a natural tooth, so that teeth made in accordance with the present invention are almost undistinguishable from natural teeth even under the most trying light conditions, for example when viewed at night by artificial light, and at the same time, even though manufactured by mass production methods, possess the lack of uniformity of natural teeth, and if desired, imitate usual defects and repair work common to natural teeth.

Other objects and advantages of the present invention will be made manifest in the following more detailed description and by reference to the accompanying drawings, wherein:

Fig. 1 is a side elevation of a tooth, for example an anterior tooth, embodying the present invention;

Fig. 2 is a front or labial view of the tooth of Fig. 1;

Fig. 3 is a vertical section on the line 3—3 of Fig. 2;

Fig. 4 is a transverse section on the line 4—4 of Fig. 3;

Fig. 5 is a vertical section substantially on the line 5—5 of Fig. 3;

Fig. 6 is a front elevation, to large scale, of an artificial tooth of a preferred construction;

Fig. 7 is a fragmentary horizontal section, to larger scale, substantially on the line 7—7 of Fig. 6;

Fig. 8 is a section generally similar to that of

Fig. 3, but illustrating a modification of the structure of Fig. 3;

Fig. 9 is a section similar to Fig. 8, but showing a further modification;

Fig. 10 is a section similar to Fig. 3, showing a still further modification;

Fig. 11 is a front elevation illustrating a denture having mounted therein a plurality of teeth embodying the present invention;

Fig. 12 is a front elevation of an artificial tooth having simulated fillings therein;

Fig. 13 is a section substantially on the line 13—13 of Fig. 12; and

Fig. 14 is a section, to very large scale, substantially in the same plane as Fig. 13, illustrating a step in the manufacture of the tooth of Fig. 12.

With reference to the following description of the improved tooth structure, it may first be stated that the improved tooth may be made in substantial accordance with usual methods employed in making artificial teeth, including the packing of suitable slip material into the cavities of complementary mould members; the closing of the mould members and subjecting them to pressure and heat; and the subsequent removal of the "green" teeth from the mould and the firing of the teeth at a temperature such as to harden, and to some extent at least, fuse the ceramic material of which the tooth is composed.

Referring to Figs. 1 to 5 of the drawings, which illustrate certain broad aspects of the invention, the numeral 1 designates the body portion of a tooth, such body portion being formed from a slip material designed to produce a body of a substantial degree of opacity, it being understood that the slip material forming the body portion may be tinted as desired, so as accurately to simulate the color of the body portion of a natural tooth.

The body portion 1 preferably has embedded therein a suitable anchorage, for example, a metal part 2, which receives a pin 2<sup>a</sup> soldered or otherwise secured to the anchorage, and by means of which the tooth may be mounted on a support, for example, a plate or bridge.

The body portion 1 has the gingival surface 3, the labial surface 4 and the lingual or pin-bearing surface 5 which extends down from the gingival surface to the usual plate-limiting boss or shoulder, and preferably tapers downwardly at its lower part to form a spur or tongue-like portion 1<sup>a</sup>, the lower end of which is substantially spaced from the incisal edge 9 of the finished tooth.

As illustrated in Figs. 1 to 5, inclusive, the incisal portion of the tooth is formed as a generally triangular mass or cap 6 of substantial depth vertically and of enamel-like material, and comprising an upwardly extending labial coating or cusp having the forward surface 7 which merges smoothly with the surface 4 of the body portion, and a lingual coating or cusp having a rear surface 8 which extends upwardly and rearwardly to a point well above the lower end of the spur 1<sup>a</sup> of the body portion, as here shown to the plate-limiting boss or shoulder of the body portion. The triangular incisal mass or cap 6 also has lateral extensions 6<sup>a</sup> and 6<sup>b</sup> (Figs. 2 and 5) which extend upwardly at opposite sides of the spur 1<sup>a</sup> of the body portion, the edges of these extensions 6<sup>a</sup> and 6<sup>b</sup> merging smoothly with the lateral edges 1<sup>m</sup> and 1<sup>n</sup> of the body portion.

From inspection of Figs. 3 and 4 it will be noted that the triangular incisal mass or cap 6 has a downwardly directed cavity forming in effect a socket for the reception of the lower part of the

spur 1<sup>a</sup>, the latter being embedded in and fused with the material forming the walls of such socket in the cap. However, as above noted, the spur 1<sup>a</sup> terminates at a substantial distance from the incisal edge 9 of the tooth, this distance, as illustrated, being two or more times the maximum horizontal thickness of the enamel at the labial side of the spur 1<sup>a</sup> and preferably exceeding one-third or even one-half of the distance between the labial surface 4 and the pin-bearing surface 5, that is to say the maximum horizontal thickness of the tooth at its upper portion.

The enamel-forming slip used in making the incisal mass or cap 6 is such that when the tooth is completed the cap transmits light much more readily than does the material of the body portion 1. In fact, the cap is completely transparent, that is to say transparent to the extent that the outlines of an object may be seen through the substance of the tooth at the incisal portion of the latter, the tooth in this respect closely simulating a usual natural tooth.

When a tooth constructed as above described is arranged in normal position so as to be viewed against the dark background of the oral cavity, light is reflected from the surface 4 of the body portion 1, the latter being substantially opaque and usually of a light color, whereas light that strikes the labial surface 7 of the cap 6 passes quite freely through the cap material and is largely absorbed by the oral cavity, so that the cap portion appears as a dark fringe bordering the incisal portion of the tooth. The spur 1<sup>a</sup> of the body portion extends downwardly into the socket cavity in the upper part of the cap 6 as above described, not only to obtain a mechanical advantage in effecting a strong union between the body portion and the cap, but for the further reason that the gradually tapering spur 1<sup>a</sup> results in a gradual screening of the light and a corresponding change in appearance from the relatively light upper portion of the tooth down toward the dark incisal edge portion, thus further simulating the appearance of the natural tooth in which the opacity gradually increases from the incisal edge toward the gingival surface and likewise inwardly from the lateral edges toward the center of the tooth.

While as illustrated in Fig. 3 the enamel forming the cap 6 terminates about midway the height of the tooth, it is contemplated that the enamel layer might be extended up even as far as the gingival surface. Thus, as shown in Fig. 10, where the tooth is otherwise like that in Fig. 3, the material forming the cap 6 is shown as extending up in a thin layer 6<sup>x</sup> covering and protecting the labial face of the body portion 1. With such an arrangement, if the enamel layer 6<sup>x</sup> be colorless but substantially transparent, the color of the body material will show through this enamel layer without substantial change except that the enamel layer imparts a bone-like or ivory luster to the entire labial surface of the tooth.

In accordance with the present invention it is also proposed to form the front or labial surface of the tooth so as closely to simulate a natural tooth by the inclusion of narrow streaks and stains of a color or appearance which visually contrasts with that of the enamel and simulates the stains and streaks common in natural teeth. With this object in view, the present invention contemplates the use of elongate masses or inserts of a material less transparent than the enamel and which may be as deeply colored as desired, these inserts being so disposed as to ex-

tend up from the incisal edge of the tooth to any desired distance and in general to extend substantially perpendicular to such edge. As illustrated in Fig. 6 the upper portions at least of the inserts 13 are located in front of the lower part of the body portion and project forwardly from the latter into the layer 7 of enamel which overlies the labial surface of the body portion. The intended effect of these inserts, at least at the translucent incisal portion of the tooth, is largely dependent upon the presence of a dark background (for example, the oral cavity or a proper masking for the supporting member of the tooth) against which to view the transparent incisal part of the tooth.

Preferably these streak simulating elements 13 take the form of elongate, triangular prisms, extending lengthwise of the tooth and desirably of slightly irregular contour so as better to simulate the irregular striations of the natural tooth. Preferably these inserts taper in width upwardly and downwardly from their mid-portions as illustrated in Fig. 6. As already stated, these streak simulating elements 13 contrast visually in appearance with the enamel; for example, they may be of a contrasting color or merely different in degree of opacity from the enamel; and one or more of such streak simulating elements may be embedded in the enamel of a tooth so as to become fused or otherwise permanently integrated with the enamel.

By making these streak simulating elements of wedge shape or triangular transverse section an indistinct or shadow effect is produced which much more closely simulates the natural tooth than would a streak simulating element of uniform transverse thickness.

In order to simulate the irregular, light-colored spots which sometimes appear in natural teeth, the present invention contemplates the interposition of bodies of material (indicated at 26 in Figs. 6, 7 and 11), usually of ceramic character, which are preferably preformed to the desired contour and size and which are inserted in the slip which forms the tooth during the moulding operation. Preferably these inserted bodies are so disposed as to be sunk partly in the material forming the body of the tooth but to project forwardly into the enamel which forms the labial surface layer and are interfused with the body and enamel layers although substantially preserving their original shapes. Such inserts, when viewed through the enamel (if made of a material which is of a light color as compared with the body of the tooth) closely simulate the light-colored, dead appearing spots often observed in natural teeth.

In Figs. 6, 7, 11, 12 and 13 the tooth of the present invention is illustrated as provided with one or more simulated fillings, for instance simulations of a porcelain or synthetic porcelain filling such as are customarily employed in repairing natural teeth. These simulated fillings 15 are preferably of a color or of optical properties slightly different from the surrounding portions of the tooth but preferably should not so differ from the tooth in appearance as to be objectionably noticeable. As it is common for a porcelain filling to bleach slightly during use, so that it appears lighter colored than the surrounding portions of the tooth, it is preferable, in accordance with this invention, to make the simulated filling 15 slightly lighter in color than the surrounding material. Thus if the simulated filling be employed in a tooth having a transparent or very translucent incisal portion 6 or labial enamel

layer 7, the simulated filling 15 may be of enamel somewhat more opaque than the main body of enamel. While it is preferred to employ this simulated filling in a tooth such as hereinabove described, wherein the incisal portion is transparent, it is obvious that such simulated filling may be applied to any type of artificial tooth.

In making a tooth having a simulated filling such as that of Fig. 12, the green tooth may be shaped to receive the filling-simulating body by the use of a mould having a properly contoured surface or the filling-receiving groove 16 (Fig. 14) may be made in the green tooth by cutting into the enamel 6, which forms the incisal edge and/or the labial layer, by the use of a suitable graving tool.

After forming this groove or notch 16, an elongate narrow layer of a stain is preferably placed therein, usually of a dark color as compared with the rest of the tooth thereby to simulate the effect of leakage around a loose or poorly fitted filling in a natural tooth. In some cases the stain 17 is disposed only in the bottom of the groove, but for pronounced effect it may cover the entire wall of the groove. After this elongate narrow layer of stain has been placed in the groove, a coating 15 of enamel forming material, usually more opaque or at least of different optical properties from the main layer of enamel, is put over the main layer of enamel, one edge 18 (Fig. 13) of said coating filling and being defined by the groove and its other margins gradually tapering and merging smoothly with the main body 6 of the enamel. Since the edge portion 18 of this filling-simulating enamel 15 completely fills the balance of the groove not occupied by the stain 17 (if the latter be used) and since the enamel is fused to the main body of enamel 6 when the tooth is fired, the stain 17 is thereby completely housed in, hermetically sealed and protected from contact with the fluids of the mouth. Such simulated fillings ordinarily contrast but slightly with the main layer of enamel in appearance and usually are substantially flush with the latter or project very slightly. However, if desired, more pronounced effects may be secured, as for instance by permitting the incisal edge of the filling material to project slightly below the incisal edge of the main body of enamel so that a distinct notch appears at their junction.

In order to provide additional color effects, the arrangement of Fig. 8 may be used, wherein the body portion of the tooth is indicated at 20 and the enamel cap at 21 (the latter having the labial surface 22, the lingual surface 23 and the incisal edge surface 19) and there is interposed between the forwardly and upwardly extending part of the cap 21 and the forward surface of the spur, a layer 25 formed from slip material which may be of the same general character as that used in the body portion or in the cap portion if desired, but which is of a different color or shade. This layer being interposed between the lower part and the body portion and the labial portion of the cap, imparts its own coloration to this part of the tooth and is found useful in obtaining some of the effects which have heretofore been accomplished but in a crude and unsatisfactory way by staining.

As shown in Fig. 9, the arrangement of Fig. 8 may further be modified by extending the material 25 upwardly in a thin layer 25<sup>x</sup> overlying the body material, and covering this thin layer

25<sup>x</sup> with an upward extension 24<sup>x</sup> of the enamel which forms the cap 21.

In Fig. 11 there is shown a denture 26 having mounted thereon a series of teeth embodying the novel features hereinabove described, and indicating the natural appearance of such teeth when mounted for use.

In the above description, when reference has been made to the "upper" or "lower" part of the tooth, it is to be understood that these and similar directional terms are used merely for convenience in description and with reference to the drawings, and without limiting intent.

Obviously other modifications and equivalent arrangements may be employed, and it is to be understood that all such modifications, substitutions of material, etc. as fall within the scope of the appended claims, are to be regarded as a part of the present invention.

I claim:

1. As an article of manufacture and sale, an artificial tooth complete and ready, when supplied to the dentist, to be incorporated, without unusual modification of structure in a denture, said tooth comprising a substantially opaque body portion and a coating of enamel fused to and overlying the incisal part at least of the labial surface of the body portion, an elongate narrow layer of stain, optically distinct from the enamel which forms said coating, located between the lingual and labial surfaces of said coating, and a body of enamel fused to said enamel coating and completely covering the stain thereby protecting the stain from contact with the fluids of the mouth.

2. As an article of manufacture and sale, an artificial tooth complete and ready to be incorporated without unusual modification of structure, in a denture, said tooth being of the kind in which a substantially opaque body has a coating of transparent enamel fused to its labial face, said tooth being characterized in having filling-simulating enamel, more opaque than the enamel coating and of small superficial extent as compared with the labial area of the tooth, fused to the enamel coating and constituting a portion of the outer surface of the tooth, and means operative to emphasize the line of junction of said filling-simulating material with the enamel coating.

3. As an article of manufacture and sale, an artificial tooth complete and ready, when supplied to the dentist, to be incorporated, without unusual modification of structure in a denture, said tooth comprising a substantially opaque body and a main layer of transparent enamel covering the labial surface of the body, a simulated filling consisting of enamel less transparent than said main layer of enamel and of an area which is small as compared with the entire labial area of the tooth, the simulated filling having an edge which is directed rearwardly and which is seated in a cavity in the labial side of the tooth, and a dark staining substance within said cavity and covered by the filling-simulating enamel, the filling-simulating enamel being fused to the main body of enamel and exposed at the outer surface of the tooth and having a contour such as to simulate a filling in a natural tooth.

4. An artificial tooth of the kind having a body portion of relatively opaque ceramic material which constitutes the major part of the tooth and enamel forming the incisal edge of the tooth, characterized in that the edge-forming enamel is an integral part of a mass of substantially

colorless enamel which is relatively more transparent than the material of the body of the tooth and which has an upward extension overlying the lower part at least of the labial surface of the body portion, said edge-forming enamel extending vertically down below the lower end of the body portion to a distance which is at least one-third of the maximum horizontal distance between the labial and lingual surfaces of the tooth and acting, when the tooth is viewed against the background of the oral cavity, to impart a dark appearance to the lower portion of the tooth, and a simulated filling of small superficial area as compared with the entire labial area of the tooth, said filling consisting of enamel of different optical properties from said incisal enamel, fused to said upward extension.

5. An artificial tooth comprising a body portion of relatively opaque material which constitutes the major part of the tooth and a body of transparent enamel forming the incisal edge portion of the tooth, characterized in that said edge-forming enamel is of such a degree of transparency as to permit the outline of an object to be seen through the substance of the tooth at its incisal portion, the vertical depth of said edge-forming enamel, between the lowest point of the body portion and the incisal edge of the tooth, exceeding one-third the maximum dis-

20 tance between the labial and lingual surfaces of the tooth whereby, when the tooth is viewed against the darkness of the oral cavity, a substantial area, adjacent to the incisal edge, appears darker than the gingival portion of the tooth, and a simulated filling of small superficial area as compared with the entire labial area of the tooth, said filling consisting of material of less transparency than the body of enamel which constitutes the incisal portion of the tooth and being fused to said incisal body of enamel.

6. An artificial tooth comprising a body portion of relatively opaque material which constitutes the major part of the tooth and an incisal mass of material which is of such a degree of transparency as to permit the outline of an object to be seen through the incisal portion of the tooth, said incisal mass terminating in an incisal edge and forming portions at least of the lateral edges of the tooth, the lower end of the body portion being fused with the material of said incisal mass, ceramic, filling-simulating material, more opaque than said incisal portion, fused with the material which forms said incisal mass, and means overlain by the filling-simulating material and effective to emphasize the junction of said filling-simulating material with said incisal mass.

SIMON MYERSON.